

Nov. 15, 1949

D. E. WEBSTER

2,488,151

METHOD OF MAKING ABRASIVE TEETH

Filed Dec. 4, 1945

2 Sheets-Sheet 1



Fig. 2



Fig. 1



Fig. 3

Fig. 4



Inventor

DUANE E. WEBSTER

384 George G. Thompson  
Attorney

Nov. 15, 1949

D. E. WEBSTER

2,488,151

METHOD OF MAKING ABRASIVE TEETH

Filed Dec. 4, 1945

2 Sheets-Sheet 2



Fig. 9



Fig. 7



Fig. 5



Fig. 6



Fig. 8

DUANE E. WEBSTER Inventor

By George Compton Jr. Attorney

## UNITED STATES PATENT OFFICE

2,488,151

## METHOD OF MAKING ABRASIVE TEETH

Duane E. Webster, Worcester, Mass., assignor to  
 Norton Company, Worcester, Mass., a corpora-  
 tion of Massachusetts

Application December 4, 1945, Serial No. 632,711

1 Claim. (Cl. 219—12)

1

The invention relates to metallurgical processes particularly for the manufacture of diamond abrasive inserts, cutting teeth, wheels and the like.

One object of the invention is to provide a method for strongly attaching a diamond impregnated piece to a holding member. Another object of the invention is to provide a method particularly useful for the manufacture of a composite abrasive article, i. e., where the complete article, be it a wheel, a band saw or any other species, consists of a quantity of diamond abrasive units.

Another object of the invention is to make articles of the class indicated cheaply and expeditiously. Another object of the invention is to make a diamond abrasive inserted tooth or the like in which the abrasive piece is secured to the backing member with a stronger union than has hitherto been found possible. Other objects will be in part obvious or in part pointed out hereinafter.

The invention accordingly consists in the features of construction, combinations of elements, arrangements of parts, and in the several steps and relation and order of each of said steps to one or more of the others thereof, all as will be illustratively described herein, and the scope of the application of which will be indicated in the following claim.

In the accompanying drawings illustrating the manufacture of a particular article by means of the process of this invention,

Figure 1 is an end elevation of the separate parts from which an abrasive tooth may be made in accordance with this invention;

Figure 2 is a plan view showing the parts of Figure 1 in assembled relation within the loop of a high frequency induction heating apparatus;

Figure 3 is a side elevation of the apparatus of Figure 2 with the parts of the tooth in position for welding;

Figure 4 is a front elevation of the same assembly as shown in Figures 2 and 3;

Figure 5 is a side view of the completed abrasive tooth;

Figure 6 is an end view of the tooth of Figure 5;

Figure 7 is a fragmentary view of a small portion of the periphery of a stone cutting disk showing a socket wherein may be inserted a tooth;

Figure 8 is a sectional view taken on the line 8—8 of Figure 7; and

Figure 9 is a side elevation of the disk with inserted abrasive teeth.

Referring first to Figure 1, a diamond abrasive

2

piece 10 may be molded to the shape shown. I provide a diamond abrasive consisting of diamonds bonded with a non-ferrous metal bond. Preferably I proceed in accordance with Reissue 5 Patent No. 21,165 to Edward Van der Pyl which describes the manufacture of diamond abrasives by mixing a quantity of crushed diamond bort with metal powder, pressing the mixture in a mold to make the desired shape, then sintering at a temperature high enough to form a strong, tough abrasive piece.

One widely used formula for diamond abrasive bodies in accordance with the Van der Pyl patent consists of 18.6% tin and 81.4% copper, by weight, in separate powders, which produces a tough but friable bond for the diamonds. The concentration of diamonds may vary, depending upon particular material to be ground, but as an illustrative example I may use 25% by volume of diamonds, the remainder metal powders, to form the bond.

I now provide a steel adapter 11 which in this case is U-shaped in cross-section or end view and has countersunk holes 12 through the legs 15 of the U, there being a total of eight of such holes. I further provide some solder or brazing material which in this illustrative example is silver solder represented by the strip 13, Figure 1. The strip 13 is cut out of sheet solder to make a nice fit in the shallow groove 14 of the piece 10.

I then assemble the parts, as well illustrated in Figures 2, 3 and 4, with the solder strip 13 in the groove 14 and between the piece 10 and the adapter 11.

35 The assembly of the abrasive piece 10 and the adapter 11 with the strip of solder between them is placed, as shown in Figures 2, 3 and 4, in a coil or loop (in this case a loop) 20 of an induction heating apparatus. It is desirable that the plane 40 of the lower edge of the loop should come just about at the top of the piece 10 and this places the strip of solder 13 just beyond the plane of the edge of the loop and not within the volume enclosed by any loop. To that end I may mount the assembly of the piece 10 and adapter 11 upon a block 21 resting on the table 22 of the induction heating machine. Furthermore, in order to have a slight pressure and a firm contact between the parts being welded or soldered together, I preferably place a weight as represented by a block 23 45 upon the top of the adapter 11. The blocks 21 and 23 are made of non-conducting or di-electric material as otherwise they would absorb power 50 from the loop 20.

With regard to the solder 13, any hard solder or brazing material can be used and this includes various brasses and various formulae for silver solder. Merely as an example, I find that a silver solder which consists of 55.82% Ag, 22.10% Cu, 17.19% Zn and 4.90% Sn, all parts by weight, gives very satisfactory results.

The loop 20 is hollow and cold water is pumped through it while the machine is in operation. Any suitable size or shape of loop or coil can be connected into the machine, the loop 20 being held in place by nuts 25 engaging threaded nipples inside the nuts which at once deliver electric energy and also cooling water. Induction heating and welding machines required for this operation are available on the market; I have obtained very satisfactory results with a machine providing 1070 British thermal units per minute or approximately 20 kilowatts at a frequency of 375,000 cycles per second.

When the parts are assembled as shown in Figures 2, 3 and 4 and the loop 20 is energized, the end of the adapter 11 adjacent the piece 12 will heat up in a matter of seconds. Actually it will be red hot in about twenty seconds. It is kept at this temperature for merely a few seconds and then the power is turned off. Care should be exercised that no metal part shall touch the loop 20 as if it does a hole will be burned in the loop 20.

Although the end of the adapter 11 adjacent the diamond abrasive piece 10 gets red hot, the diamond abrasive piece 10 which is definitely in the high frequency electromagnetic field does not get red hot and, in fact, remains comparatively cool. This is the important feature which enables me to make satisfactory pieces by this welding or soldering or brazing process since were the piece 10 to get red hot during the welding operation it would be ruined as an abrasive. The outer layer of diamonds in the piece 10 would burn if it were red hot.

There are two phenomena involved in induction heating. One is hysteresis and the other is eddy currents. Around every conductor carrying electricity is a magnetic field. If the current is alternating, the magnetic field reverses with the alternation. A reversing magnetic field generates an electromotive force in any conductor located in said field. Such electromotive force will create eddy currents in a solid block of conducting material. On the other hand, if the material is paramagnetic, in addition to the eddy currents due to the conductivity of the material there is the phenomenon of hysteresis, which constitutes the movement of the molecules of the material as they try to adjust themselves parallel to the magnetic lines of force which in this case change their direction 375,000 times a second.

Furthermore, the heating effect due to the eddy currents is less with high conductivity material such as copper than it is with relatively poor conductors such as iron. For these reasons it is found that the lower end of the adapter 11 can be heated red hot while the diamond abrasive piece 10 is still relatively cold.

Figures 5 to 9 illustrate the manufacture of a stone cutting disk 30 having abrasive teeth 31, each tooth consisting of a diamond abrasive piece 10 and an adapter 11. The disk 30 is made of steel and in an actual case was 90 inches in diameter. Recesses 33 are milled in each side of the disk at spaced intervals around its periphery, a pair of recesses 33 being opposite each other, all as clearly shown in the drawings. Through the connecting

web 34 connecting a pair of recesses 33 are drilled four holes 35 spaced the same as the countersunk holes 12. Enough abrasive teeth 31 are provided so that the adapters thereof will fill all of the recesses 33. Then the teeth are placed in position as shown and riveted to the disk 30 by rivets passing through the holes 35 and headed over in the countersinks of the holes 12. In this manner a very strong and rigid abrasive wheel is produced which is useful as a stone cutting saw to cut large blocks of granite or other hard rock.

Diamond abrasives are used only to grind hard materials because it would be extravagant to use them where aluminous abrasives or carbide abrasives would suffice. For certain materials which may be hard but not too tough, diamond abrasive bonded with resinoid is preferred. But in the case of certain hard and tough materials, such as granite, diamond abrasive bonded with metal bond is found to give the best results. Diamond abrasive bonded with metal bond is hard, tough and strong. It will grind granite readily, but a great deal of power is consumed in the operation. In the use of this enormous saw 30, which is 7½ feet in diameter, the abrasive pieces 10 are forced into the granite with great pressure. This pressure is trying to rip the pieces 10 from the adapters 11. A surer test of the strength of the metallurgical union could hardly be devised. It has been found that the abrasive teeth made in accordance with this invention survive this test and the granite saw 30 is effective to cut granite.

The process of the invention may be used for securing diamond abrasive pieces bonded with non-ferrous metal bond to iron or steel adapters or directly to iron or steel circular saws or iron or steel band saws or, in fact, wherever it is desired to attach such non-ferrous metal bonded diamond abrasive pieces to anything made of iron or steel.

It will thus be seen that there has been provided by this invention a method in which the various objects hereinabove set forth together with many thoroughly practical advantages are successfully achieved. As various possible embodiments might be made of the mechanical features of the above invention and as the art herein described might be varied in various parts, all without departing from the scope of the invention, it is to be understood that all matter hereinbefore set forth or shown in the accompanying drawings is to be interpreted as illustrative and not in a limiting sense.

I claim:

55 The method of attaching a diamond abrasive piece consisting of diamonds bonded with a metal bond the major part of which is copper to a piece of ferrous metal, including the step of forming on the diamond abrasive piece a surface and forming on the piece of ferrous metal a surface which surfaces fit each other nicely; the step of placing a flat strip of solder between said surfaces said strip of solder contacting each surface so that said surfaces are facing each other with the strip of solder in between them; the step of pressing said surfaces towards each other; the step of placing the pieces with relation to a loop of a high frequency induction heating machine so that the strip of solder is just beyond the plane of the 60 edge of the loop and not within the volume enclosed by any loop but with part of the piece of ferrous metal adjacent said strip of solder within the said volume enclosed by the loop; the step of energizing the loop of the machine until the 65 piece of ferrous metal in said volume is red hot

and discontinuing the energization before the diamond abrasive piece becomes red hot, the surfaces being pressed towards each other while the piece of ferrous metal is red hot.

DUANE E. WEBSTER.

REFERENCES CITED

The following references are of record in the file of this patent:

UNITED STATES PATENTS

| Number     | Name           | Date           |
|------------|----------------|----------------|
| Re. 21,165 | Van Der Pyl    | July 25, 1939  |
| 1,996,598  | Taylor         | Apr. 2, 1935   |
| 2,200,281  | Koebel         | May 14, 1940   |
| 2,216,908  | De Bats        | Oct. 8, 1940   |
| 2,233,176  | Melton et al.  | Feb. 25, 1941  |
| 2,299,207  | Bevillard      | Oct. 20, 1942  |
| 2,316,506  | Doelker et al. | Apr. 13, 1943  |
| 2,358,459  | Kelleher       | Sept. 19, 1944 |

FOREIGN PATENTS

| Number  | Country       | Date          |
|---------|---------------|---------------|
| 286,823 | Great Britain | Mar. 15, 1928 |

OTHER REFERENCES

- 10 "High Frequency Brazing" in "The Welding Encyclopedia," Eleventh edition, 1943, published by Welding Engineer Publishing Co., Chicago, Illinois, pages 691 and 694.
- 10 "Product Engineering," February 1943, pages 102-104.
- 10 "Carbide Tools Tipped by Induction Brazing," by Paul Miller in "American Machinist," October 14, 1943, pages 106, 107.
- 15 Curtis, "High-Frequency Induction Heating," 1944, pages 114 and 115, McGraw-Hill Book Company, Inc., New York, New York.